

## UNITED STATES PATENT OFFICE.

WLADISLAUS RAKOWSKI, OF PHILADELPHIA, PENNSYLVANIA.

## BINDER FOR COAL BRIQUETTES AND THE LIKE.

No Drawing.

Application filed June 2, 1923. Serial No. 643,071.

My invention relates to new and useful improvements in a binder for coal briquettes and the like, and has for its primary object to use a siccative oil for holding together 5 fragments of different sizes of coal waste or refuse, coke-braize or other substances having either combustible or non-combustible properties.

Another object of the invention is to use 10 in conjunction with the siccative oil as a binder, in some cases, a suitable adhesive to primarily hold the particles together so that the object produced may be handled prior to the drying process.

Another object of the invention consists 15 of a process or method for manufacturing articles with the use of the binder above mentioned which comprises the mixing of the binder with fragments or particles of 20 coal, coke-braize, sand or the like, then subjecting the mass to pressure in a mold and then heated while in the mold to dry the same and produce an exceedingly hard product which, in the case of a fuel, may afterwards be broken so as to correspond with 25 the ordinary or standard sizes of coal.

A further object of the invention is to provide an additional step in the process above mentioned in some particular cases 30 which consists in adding or mixing with the mass a suitable adhesive to act as a temporary binder prior to the heating or hardening action.

In order to make coal briquettes like 35 those on the market at the present, I add, if coarse material is used, to the siccative oil moistened mass, a suitable adhesive, since briquettes of coarse material, held together by a siccative oil only, are weak and 40 are likely to fall apart when being moved from the press to the drying room, but the use of the adhesive overcomes this difficulty and, when dried thoroughly in a hot room, the siccative will effect such hard product, 45 that it will not fall apart during handling and will not disintegrate when burned as a fuel, until the combustible particles have been consumed. If the prepared mass consists of very fine fragments and is subjected 50 to considerable pressure, the addition of an adhesive substance is not needed.

In carrying out my invention, I take one hundred pounds of coal culm, coke-braize or other fuel refuse or waste and moisten 55 the same with two quarts of unaltered siccative

oil, examples of which are cotton seed and linseed oils, next a quantity of this mass is placed in a mold of any desirable size or shape where the contents are subjected to pressure and while the mass is in the mold 60 heat is applied for drying it and the resultant product will be very hard and when made in large pieces the same may afterwards be broken into fragments in sizes corresponding to the ordinary or standard 65 anthracite coal sizes and generally known as egg, stove, nut, pea, etc.

A product produced as above set forth in addition to being very hard, is water proof, will not disintegrate or crumble while being 70 burned, until the products of combustion have been consumed, and will not soil the hands.

Of course I do not wish to be limited to the exact details of construction as herein 75 shown as these may be varied within the limits of the appended claims without departing from the spirit of my invention.

Having thus fully described my invention, what I claim as new and useful is:— 80

1. The process of producing briquettes which comprises adding to body material, in a divided state, a sufficient quantity of an unaltered siccative oil to moisten the same, compressing the mass, and heating 85 the same to dryness while under pressure.

2. The process of producing briquettes which comprises adding to body material, in a divided state, a sufficient quantity of unaltered linseed oil to moisten the same, 90 compressing the mass, and heating the same to dryness while under pressure.

3. The process of producing briquettes which comprises adding to coal or coke refuse or similar combustible material, in a 95 divided state, a sufficient quantity of an unaltered siccative oil to moisten the same, compressing the mass, and heating the same to dryness while under pressure.

4. The process of producing briquettes 100 which comprises adding to coal or coke refuse, or similar combustible material, in a divided state, an adhesive, and a sufficient quantity of an unaltered siccative oil to moisten the same, compressing the mass, and heating the same to dryness while under pressure.

In testimony whereof, I have hereunto affixed my signature.

WLADISLAUS RAKOWSKI.